



US008048397B2

(12) **United States Patent**  
**Chen et al.**

(10) **Patent No.:** **US 8,048,397 B2**  
(b5) **Date of Patent:** **\*Nov. 1, 2011**

(54) **LASER-BASED METHOD FOR MAKING FIELD EMISSION CATHODE**

(75) Inventors: **Zhuo Chen**, Beijing (CN); **Chun-Xiang Luo**, Beijing (CN); **Kai-Li Jiang**, Beijing (CN); **Shou-Shan Fan**, Beijing (CN)

(73) Assignees: **Tsinghua University**, Beijing (CN); **Hon Hai Precision Industry Co., Ltd.**, Tu-Cheng, New Taipei (TW)

(\*) Notice: Subject to any disclaimer, the term of this patent is extended or adjusted under 35 U.S.C. 154(b) by 941 days.

This patent is subject to a terminal disclaimer.

(21) Appl. No.: **11/982,674**

(22) Filed: **Nov. 2, 2007**

(65) **Prior Publication Data**

US 2008/0268739 A1 Oct. 30, 2008

(30) **Foreign Application Priority Data**

Dec. 22, 2006 (CN) ..... 2006 1 0157895

(51) **Int. Cl.**

**D01C 5/00** (2006.01)

(52) **U.S. Cl.** ..... **423/447.3; 423/445 B; 977/742; 977/843; 427/586; 438/20**

(58) **Field of Classification Search** ..... None  
See application file for complete search history.

(56) **References Cited**

U.S. PATENT DOCUMENTS

2,549,298 A 4/1951 Donegan  
4,226,900 A 10/1980 Carlson et al.  
4,682,075 A 7/1987 Nelson et al.

|              |         |                |
|--------------|---------|----------------|
| 4,702,558 A  | 10/1987 | Coles et al.   |
| 5,154,945 A  | 10/1992 | Baldwin et al. |
| 5,288,558 A  | 2/1994  | Nothe          |
| 6,444,400 B1 | 9/2002  | Cloots et al.  |
| 6,869,479 B2 | 3/2005  | Shafeev et al. |
| 6,917,058 B2 | 7/2005  | Niigaki et al. |
| 7,357,691 B2 | 4/2008  | Liu et al.     |
| 7,448,931 B2 | 11/2008 | Liu et al.     |
| 7,682,658 B2 | 3/2010  | Jiang et al.   |

(Continued)

FOREIGN PATENT DOCUMENTS

JP 2005-239494 9/2005

(Continued)

OTHER PUBLICATIONS

Chen et al (Applied Physics Letters 90, 133108 (2007).\*)

(Continued)

*Primary Examiner* — David Turocy  
*Assistant Examiner* — Joel Horning  
(74) *Attorney, Agent, or Firm* — Altis Law Group, Inc.

(57) **ABSTRACT**

A method for making a field emission cathode includes the steps of: (a) providing a substrate having a first substrate surface and a second substrate surface opposite to the first substrate surface; (b) forming a conductive film on the first substrate surface; (c) forming a catalyst film on the conductive film, the catalyst film including carbonaceous material; (d) flowing a mixture of a carrier gas and a carbon source gas over the catalyst film; (e) focusing a laser beam on the catalyst film and/or on the second substrate surface to locally heat the catalyst to a predetermined reaction temperature; and (f) growing an array of the carbon nanotubes via the catalyst film to form a field emission cathode.

**17 Claims, 2 Drawing Sheets**



## U.S. PATENT DOCUMENTS

7,771,698 B2 8/2010 Chen et al.  
7,780,940 B2 8/2010 Chen et al.  
7,820,133 B2 10/2010 Chen et al.  
2001/0003642 A1 6/2001 Chang et al.  
2001/0010892 A1 8/2001 Mori  
2002/0061362 A1 5/2002 Chiavarotti et al.  
2002/0081397 A1 6/2002 McGill et al.  
2002/0160111 A1 10/2002 Sun et al.  
2003/0130114 A1 7/2003 Hampden-Smith et al.  
2004/0060477 A1 4/2004 Iwaki et al.  
2004/0209385 A1 10/2004 Liu et al.  
2004/0253758 A1 \* 12/2004 Jung et al. .... 438/22  
2005/0000438 A1 \* 1/2005 Lim et al. .... 118/722  
2005/0052127 A1 3/2005 Sakata et al.  
2005/0113509 A1 5/2005 Tazzia  
2005/0118525 A1 \* 6/2005 Kim et al. .... 430/200  
2006/0104890 A1 5/2006 Harutyunyan et al.

2006/0147848 A1 \* 7/2006 Han et al. .... 430/327  
2006/0238095 A1 \* 10/2006 Nam .... 313/311  
2006/0263524 A1 11/2006 Jiang et al.  
2008/0233402 A1 9/2008 Carlson et al.  
2008/0268739 A1 10/2008 Chen et al.

## FOREIGN PATENT DOCUMENTS

TW 200634171 10/2006

## OTHER PUBLICATIONS

Kinghong Kwok, Wilson K.S. Chiu. "Growth of carbon nanotubes by open-air laser-induced chemical vapor deposition". Carbon, 2005, vol. 43, p. 437-446.  
Composition and Properties of Oil Well Drilling Fluids, 4th Ed., Gray and Darley, Gulf Publishing Company, 1981, p. 9.

\* cited by examiner

providing a substrate having a first substrate surface and a second substrate surface opposite to the first substrate surface

forming a conductive film on the first substrate surface

forming a catalyst film on the conductive film, the catalyst film including carbonaceous material

flowing a mixture of a carrier gas and a carbon source gas over the catalyst film

focusing a laser beam on the catalyst film and/or on the second substrate surface to locally heat the catalyst film to a predetermined reaction temperature

growing an array of the carbon nanotubes via the catalyst film to form a field emission cathode

FIG. 1



**FIG. 2**



**FIG. 3**

## 1

LASER-BASED METHOD FOR MAKING  
FIELD EMISSION CATHODE

## RELATED APPLICATIONS

This application claims all benefits accruing under 35 U.S.C. §119 from China Patent Application No. 200610157895.5, filed on 2006 Dec. 22 in the China Intellectual Property Office, the contents of which are hereby incorporated by reference. This application is related to commonly-assigned applications entitled, "LASER-BASED METHOD FOR MAKING FIELD EMISSION CATHODE", Ser. No. 11/982,486, filed on 2007 Nov. 2; "LASER-BASED METHOD FOR GROWING ARRAY OF CARBON NANOTUBES", 11/982,485, filed on 2007 Nov. 2; "LASER-BASED METHOD FOR GROWING ARRAY OF CARBON NANOTUBES", Ser. No. 11/982,517, filed on 2007 Nov. 2; "LASER-BASED METHOD FOR GROWING ARRAY OF CARBON NANOTUBES", Ser. No. 11/982,667, filed on 2007 Nov. 2; and "LASER-BASED METHOD FOR GROWING ARRAY OF CARBON NANOTUBES", Ser. No. 11/982,669, filed on 2007 Nov. 2; and "LASER-BASED METHOD FOR GROWING ARRAY OF CARBON NANOTUBES", Ser. No. 11/982,489, filed on 2007 Nov. 2. Disclosures of the above-identified applications are incorporated herein by reference.

## BACKGROUND

## 1. Field of the Invention

The invention relates generally to methods for making a field emission cathode and, particularly, to a laser-based method for making a carbon nanotube-based field emission cathode.

## 2. Discussion of Related Art

Carbon nanotubes are a novel carbonaceous material discovered and reported in an article by Sumio Iijima, entitled "Helical Microtubules of Graphitic Carbon" (Nature, Vol. 354, Nov. 7, 1991, pp. 56-58). Carbon nanotubes can transmit an extreme high electrical current and emit electrons at a very low voltage of less than 100 volts, which make it a very promising potential material for field emission applications.

Generally, the carbon nanotubes used for field emission are produced by arc discharge method or chemical vapor deposition method. The method for applying carbon nanotubes in field emission includes the steps of: printing a patterned layer of conductive grease on a conductive base with a predetermined quantity of carbon nanotubes dispersed therein and treating the layer of grease by peeling parts of the grease to expose ends of the carbon nanotubes to emit electrons. However, the step of peeling quite often destroys the carbon nanotubes. Moreover, the carbon nanotubes for emitting electrons, generally, lie on the conductive base. Thus, the field emission efficiency thereof is relatively low, and the stability thereof is less than desired.

What is needed, therefore, is to provide a laser-based method for making a carbon nanotube-based field emission cathode in which the above problems are eliminated or at least alleviated.

## SUMMARY

A method for making a field emission cathode includes the steps of: (a) providing a substrate having a first substrate surface and a second substrate surface opposite to the first substrate surface; (b) forming a conductive film on the first substrate surface; (c) forming a catalyst film on the conductive film, the catalyst film including a carbonaceous material;

## 2

tive film, the catalyst film including carbonaceous material; (d) flowing a mixture of a carrier gas and a carbon source gas over the catalyst film; (e) focusing a laser beam on the catalyst film and/or on the second substrate surface to locally heat the catalyst film to a predetermined reaction temperature; and (f) growing an array of the carbon nanotubes via the catalyst film to form a field emission cathode.

Other advantages and novel features of the present method for making a field emission cathode will become more apparent from the following detailed description of present embodiments when taken in conjunction with the accompanying drawings.

## BRIEF DESCRIPTION OF THE DRAWINGS

Many aspects of the present method for making a field emission cathode can be better understood with reference to the following drawings. The components in the drawings are not necessarily to scale, the emphasis instead being placed upon clearly illustrating the principles of the present laser-based method for making a field emission cathode.

FIG. 1 is a flow chart of a laser-based method for making a field emission cathode, in accordance with a present embodiment;

FIG. 2 shows a Scanning Electron Microscope (SEM) image of a carbon nanotube-based field emission cathode formed by the method of FIG. 1; and

FIG. 3 shows a Scanning Electron Microscope (SEM) image of a patterned carbon nanotube-based field emission cathode formed by the method of FIG. 1.

Corresponding reference characters indicate corresponding parts throughout the several views. The exemplifications set out herein illustrate at least one preferred embodiment of the present laser-based method for making a field emission cathode, in at least one form, and such exemplifications are not to be construed as limiting the scope of the invention in any manner.

## DETAILED DESCRIPTION OF PREFERRED EMBODIMENTS

Reference will now be made to the drawings to describe, in detail, embodiments of the present laser-based method for making a field emission cathode.

Referring to FIG. 1, the laser-based method for making a field emission cathode includes the following steps: (a) providing a substrate having a first substrate surface and a second substrate surface opposite to the first substrate surface; (b) forming a conductive film on the first substrate surface; (c) forming a catalyst film on (e.g., directly on/in contact with) the conductive film, the catalyst film including a carbonaceous material; (d) flowing a mixture of a carrier gas and a carbon source gas over the catalyst film; (e) focusing at least one laser beam on the catalyst film and/or on the second substrate surface to locally heat the catalyst to a predetermined temperature; and (f) growing, via the catalyst film, an array of the carbon nanotubes to form a field emission cathode.

In step (a), the substrate is, advantageously, made of a heat-resistant material (e.g., high-melting point, chemically durable), which can tolerate the high reaction temperature (e.g., upwards of about 600° C.). It is to be understood that depending on different applications, the material of the substrate could be selected from an opaque or transparent material, e.g., an opaque material such as silicon, silicon dioxide,

or a metal for semiconductor electronic devices, or a transparent material such as a glass and plastic material for flat displays.

In step (b), the conductive film usefully is uniformly disposed (e.g., in terms of composition and/or thickness) on the first substrate surface by means of thermal deposition, electron-beam deposition, and/or sputtering. Rather usefully, the material of the conductive film is indium tin oxide film. The width of the conductive film is in the approximate range from 10 to 100 nanometers. Quite suitably, the width of the conductive film is 30 nanometers. It is noted that step (b) is provided as part of the process for making a field emission cathode, since the conductive film is used to conduct electrons and thereby facilitate a connection to an external electrical source. Essentially, the conductive film enables electrons to reach the carbon nanotubes in the grown carbon nanotube array, electrons that can then be emitted by the carbon nanotubes.

Step (c) includes the substeps of: (c1) providing a mixture of a dispersant and a carbonaceous material; (c2) combining the mixture with a solvent to form a solution; (c3) ultrasonically agitating the solution to promote the dispersion of the carbonaceous material therein; (c4) adding a soluble catalyst material into the dispersed solution to form a catalyst solution; (c5) coating the catalyst solution on the conductive film; and (c6) baking the substrate to form thereon a catalyst film that includes carbonaceous material.

In step (c1), the carbonaceous material can usefully be selected from carbon black (CB) and/or graphite. The dispersant is used for uniformly dispersing the carbonaceous material. Rather suitably, the dispersant is sodium dodecyl benzene sulfonate (SDBS). A weight ratio of the dispersant to the carbonaceous material is, advantageously, in the approximate range from 1:2 to 1:10. In step (c2), the solvent is, opportunely, water or ethanol. In one useful embodiment, an amount of SDBS in the range of about 0~100 mg (beneficially, a measurable amount of dispersant (i.e., above about 0 mg) is employed) and an amount of CB of about 100~500 mg are mixed into a volume of ethanol of about 10~100 ml to form the solution. Quite usefully, the solution is formed by combining about 50 mg of SDBS and about 150 mg of CB into about 40 ml of ethanol.

In step (c3), the solution can be sonicated (i.e., subjected to ultrasound) for, e.g., about 5 to 30 minutes to uniformly disperse the first carbonaceous material in the solution. In step (c4), the soluble catalyst material can, rather appropriately, include one or more metallic nitrate compounds selected from a group consisting of magnesium nitrate ( $Mg(NO_3)_2 \cdot 6H_2O$ ), iron nitrate ( $Fe(NO_3)_3 \cdot 9H_2O$ ), cobalt nitrate ( $Co(NO_3)_2 \cdot 6H_2O$ ), nickel nitrate ( $Ni(NO_3)_2 \cdot 6H_2O$ ), and any combination thereof. In one useful embodiment, after being treated with ultrasound for about 5 minutes,  $Fe(NO_3)_3 \cdot 9H_2O$  and  $Mg(NO_3)_2 \cdot 6H_2O$  is added to the solution, thereby forming the catalyst solution. Quite usefully, the catalyst solution includes about 0.01~0.5 Mol/L magnesium nitrate and about 0.01~0.5 Mol/L iron nitrate.

In step (c5), the catalyst solution is, beneficially, spin coated on the substrate at a rotational speed of about 1000~5000 rpm. Quite suitably, the rotational speed for spin coating is about 1500 rpm. In step (c6), the substrate, with the catalyst solution coated thereon, is baked at about 60~100°C. for 10 min~1 hr. It is to be understood that the baking process is used to vaporize the solvent in the solution and accordingly form the catalyst film on the conductive film containing carbonaceous material. The width of the catalyst film is in the approximate range from 10 to 100 micrometers.

In step (d), a carbon source gas, which is mixed with a carrier gas, is flown over/adjacent the catalyst film for growing carbon nanotubes. In one useful embodiment, the carbon source gas and the carrier gas are directly introduced, in open air, by a nozzle to an area adjacent to the catalyst film. That is, the method can be operated without a closed reactor and/or without being under a vacuum. The carrier gas can, beneficially, be nitrogen ( $N_2$ ) and/or a noble gas. The carbon source gas can, advantageously, be ethylene ( $C_2H_4$ ), methane ( $CH_4$ ), acetylene ( $C_2H_2$ ), ethane ( $C_2H_6$ ), or any combination thereof. Quite suitably, the carrier gas is argon (Ar), and the carbon source gas is acetylene. A ratio of the carrier gas flow-rate to the carbon source gas flow-rate is, opportunely, adjusted to be in an approximate range from 5:1 to 10:1. Quite usefully, the argon flow-rate is 200 sccm (Standard Cubic Centimeter per Minute), and the acetylene flow-rate is 25 sccm.

In step (e), the laser beam can be generated by a laser beam generator (e.g., a carbon dioxide laser, an argon ion laser, etc.). A power of the laser beam generator is in the approximate range from above about 0 W (Watt) (i.e., a measurable amount of power) to ~5 W. Quite usefully, a carbon dioxide laser of 470 mW is used for generating the laser beam. The laser beam generator further includes at least one lens for focusing laser beams generated by the laser beam generator. It is to be understood that the focused laser beam could be employed to directly irradiate on the catalyst film to heat the catalyst to a predetermined reaction temperature along a direction vertical/orthogonal or oblique to the substrate (i.e., the surface of the substrate upon which the array is grown). When the substrate is transparent material, it is to be understood that the focused laser beam could be employed to irradiate directly on the second substrate surface, and the substrate could transfer the heat to the catalyst film. The transferred heat would quickly to heat the catalyst to a predetermined reaction temperature along a direction vertical or oblique to the substrate. The heat transfer direction/angle would depend upon such factors as the beam angle relative to the substrate and the crystallography and/or morphology of the substrate. As a result of such various operating parameters, the method can be operated in open air without heating the entire substrate to meet a reaction temperature for synthesizing carbon nanotubes. That is, the operation and cost of the present method is relatively simple and low compared to conventional methods.

In step (e), when the focused laser beam is irradiated on the second substrate surface, laser-intensity-induced damage to the newly grown CNTs on the first surface side of the substrate can thereby be effectively avoided. Moreover, the laser beam will not directly react with the carbon source gas nor have an impact on any of the properties of the gas. Thus, the laser beam cannot undermine the growth of carbon nanotubes arrays.

In step (f), due to catalyzing by the catalyst film, the carbon source gas supplied over the catalyst film is pyrolyzed in a gas phase into carbon units ( $C=C$  or  $C$ ) and free hydrogen ( $H_2$ ). The carbon units are absorbed on a free surface of the catalyst film and diffused thereinto. When the catalyst film becomes supersaturated with the dissolved carbon units, carbon nanotube growth is initiated. As the intrusion of the carbon units into the catalyst film continues, an array of carbon nanotubes is formed, extending directly from the catalyst film. The additional hydrogen produced by the pyrolyzed reaction can help reduce the catalyst oxide and thus activate the catalyst. As such, the growth speed of the carbon nanotubes is increased, and the achievable height of the array of the carbon nanotubes is enhanced.

It is noted that the carbonaceous material in the catalyst film employed in the method has the following virtues. Firstly, the carbonaceous material will absorb laser light and thus facilitate heating of the catalyst to enable carbon nanotube growth. Secondly, the carbonaceous material will attenuate the laser field and avoid damaging the newly grown carbon nanotubes with the otherwise intense laser. Additionally, the carbonaceous material will release carbon atoms to promote the nucleation of carbon nanotubes, when irradiated by a given laser beam. Finally, because of the initial presence of the carbon in the catalyst film, the supersaturation point for carbon therein will be reached sooner, permitting carbon nanotube growth to start sooner than might otherwise be possible. As such, the predetermined reaction temperature for locally heating the catalyst film by laser beam can be less than ~600° C.

Referring to FIG. 2, a carbon nanotube-based field emission cathode manufactured by the present method is shown. The carbon nanotube-based field emission cathode is synthesized by irradiating the focused laser beam on the catalyst film formed on a glass substrate for about 5 seconds. A diameter of the focused laser beam is in the approximate range from 50 to 200 micrometers. The field emission cathode includes a substrate, a conductive film serving as an electrode film and an array of carbon nanotubes serving as emitters. The formed array of carbon nanotubes, in this example, manifests a hill-shaped. The diameter of the hill is in the approximate range from 50 to 80 micrometers. The maximum height of the hill is in the approximate range from 10 to 20 micrometers. The diameter of each carbon nanotube is in the approximate range from 40 to 80 nanometers.

FIG. 3 shows a patterned carbon nanotube-based field emission cathode manufactured by the present method is shown. The patterned carbon nanotube-based field emission cathode is synthesized by irradiating a laser beam on a predetermined pattern to selectively heat the film of carbonaceous catalyst to the reaction temperature, thereby growing a patterned array of the carbon nanotubes via/from the catalyst film to form a patterned field emission cathode. The patterned field emission cathode includes a plurality of field emission cathodes arranged in the same substrate to a predetermined pattern. Each field emission cathode includes a carbon nanotube array.

It is noted that the present method can synthesize a large area array of carbon nanotubes by scanning the laser beam on a large area substrate and that the properties of carbon nanotubes used for field emission cathode thus produced are able to be closely controlled and thereby be essentially uniform.

Compared with conventional arc discharge method or chemical vapor deposition method, the carbon nanotubes used for field emission prepared by the methods in the described embodiments are vertical to the conductive base, which can increase the field emission efficiency and the field emission stability. Furthermore, the carbonaceous material in the catalyst film employed in the method has the following virtues. Firstly, the carbonaceous material will absorb laser light and thus facilitate heating of the catalyst to enable carbon nanotube growth. Secondly, the carbonaceous material will attenuate the laser field and avoid damaging the newly grown carbon nanotubes with the otherwise intense laser. Additionally, the carbonaceous material will release carbon atoms to promote the nucleation of carbon nanotubes, when irradiated by laser beam. Finally, because of the initial presence of the carbon in the catalyst film, the supersaturation point for carbon therein will be reached sooner, permitting carbon nanotube growth to start sooner than might otherwise be possible. As such, the predetermined reaction temperature

for locally heating the catalyst film by laser beam can be less than ~600° C. What is more, the methods in the described present embodiments employ a focused laser beam, which irradiates on the second substrate surface. Such laser beam usage can effectively avoiding damaging, by intense laser, the newly grown CNTs on the first surface side of the substrate. Moreover, the laser beam will not directly react with the carbon source gas and will not have an impact on the properties of the gas. Thus, the laser beam will not undermine the growth of carbon nanotubes arrays. Moreover, the present method for growing carbon nanotubes used for field emission can proceed in open air, without a closure reactor and/or vacuum conditions. For all of the various reasons provided, the operation of the present method is relatively simple, and the resultant cost thereof is reasonably low, compared to conventional methods.

Finally, it is to be understood that the above-described embodiments are intended to illustrate rather than limit the invention. Variations may be made to the embodiments without departing from the spirit of the invention as claimed. The above-described embodiments illustrate the scope of the invention but do not restrict the scope of the invention.

What is claimed is:

1. A method for making a field emission cathode, comprising the steps of:
  - (a) providing a substrate having a first substrate surface and a second substrate surface opposite to the first substrate surface;
  - (b) forming a conductive film on the first substrate surface;
  - (c) forming a catalyst film on the conductive film, the catalyst film comprising a carbonaceous material comprising at least one of carbon black and graphite;
  - (d) flowing a mixture of a carrier gas and a carbon source gas over the catalyst film;
  - (e) focusing a laser beam on at least one of the catalyst film and the second substrate surface to locally heat the catalyst film to a predetermined reaction temperature; and
  - (f) growing an array of the carbon nanotubes via the catalyst film to form a field emission cathode.
2. The method as claimed in claim 1, wherein step (c) further comprises the substeps of:
  - (c1) providing a mixture of a dispersant;
  - (c2) combining the mixture with a solvent to form a solution;
  - (c3) ultrasonically agitating the solution to promote dispersing of the carbonaceous material therein;
  - (c4) adding a soluble catalyst material into the dispersed solution to form a catalyst solution;
  - (c5) coating the catalyst solution on the conductive film; and
  - (c6) baking the substrate to form thereon a catalyst film including the carbonaceous material.
3. The method as claimed in claim 2, wherein in step (c1), the dispersant comprises sodium dodecyl benzene sulfonate.
4. The method as claimed in claim 2, wherein in step (c1), a weight ratio of the dispersant to the carbonaceous material is in the approximate range from 1:2 to 1:10.
5. The method as claimed in claim 2, wherein in step (c2), the solvent comprises at least one of water and ethanol.
6. The method as claimed in claim 2, wherein in step (c4), the soluble catalyst material comprises a mixture of magnesium nitrate and at least one material selected from the group consisting of iron nitrate, cobalt nitrate, and nickel nitrate.
7. The method as claimed in claim 2, wherein a thickness of the catalyst film is in the approximate range from 10 to 100 micrometers.

8. The method as claimed in claim 1, wherein the material of the conductive film is indium tin oxide film.

9. The method as claimed in claim 8, wherein a thickness of the conductive film is in the approximate range from 10 to 100 nanometers.

10. The method as claimed in claim 1, wherein the carbon source gas is comprised of at least one gas selected from the group consisting of ethylene, methane, acetylene, and ethane.

11. The method as claimed in claim 1, wherein the carrier gas is comprised of at least one of nitrogen gas and a noble gas.

12. The method as claimed in claim 1, wherein a ratio of a carrier gas flow-rate to a carbon source gas flow-rate is in the approximate range from 5:1 to 10:1.

13. The method as claimed in claim 1, wherein the substrate is comprised of at least one material selected from the group consisting of silicon, silicon dioxide, a metal, a glass, and a plastic material.

14. The method as claimed in claim 1, wherein in step (e), the laser beam is generated by a laser generator selected from one of a carbon dioxide laser and an argon ion laser.

15. The method as claimed in claim 14, wherein the laser generator further comprises a lens for focusing the laser beam.

16. The method as claimed in claim 1, wherein a diameter of the focused laser is in the approximate range from 50 to 200 micrometers.

17. A method for making a patterned field emission cathode, comprising the steps of:

- (a) forming a conductive layer on a substrate;
- (b) applying a carbonaceous catalyst film comprising at least one of carbon black and graphite onto the conductive layer;
- (c) supplying a flow of a reactant gas containing a carbon source gas over the carbonaceous catalyst film;
- (d) irradiating a laser beam in a predetermined pattern to selectively heat the carbonaceous catalyst film to the reaction temperature; and
- (e) growing a patterned array of the carbon nanotubes via the carbonaceous catalyst film to form a patterned field emission cathode.

\* \* \* \* \*